# EUROPEAN PATENT SPECIFICATION

(11) **EP 0 309 159 B1**
(45) Date of publication and mention of the grant of the patent: **24.03.1993**
(21) Application number: 88308568.0
(22) Date of filing: 16.09.1988
(51) Int. Cl.: G03C 7/26, G03C 7/38

(54) **Photographic recording material comprising a dye image-forming coupler compound**
Photographisches Eintragungsmaterial, enthaltend farbbildende Kupplerverbindungen
Matériau photographique d'enregistrement comprenant des composés copulants formant une image couleur

(30) Priority: 21.09.1987 US 99176
(43) Date of publication of application: 29.03.1989
(73) Proprietor: EASTMAN KODAK COMPANY (a New Jersey corporation), Rochester, New York 14650 (US)
(72) Inventor: Merkel, Paul Barrett c/o EASTMAN KODAK COMPANY, Rochester New York 14650 (US); Giacherio, David James c/o EASTMAN KODAK COMPANY, Rochester New York 14650 (US)
(74) Representative: Baron, Paul Alexander Clifford

(56) References cited:
- EP-A- 0 264 083
- EP-A- 0 270 341
- DD-A- 231 664
- CHEMICAL ABSTRACTS, vol. 68, no. 18, 1968, page 8003, abstract no. 83108u, Columbus, Ohio, US
- PATENT ABSTRACTS OF JAPAN, vol. 9, no. 72 (P-345)[1795], 2nd April 1985

## Description

This invention relates to a color photographic silver halide recording material. In particular, the invention relates to an improved photographic recording material comprising a dye image-forming coupler compound.

Color photographic recording materials generally contain silver halide emulsion layers sensitized to each of the blue, green and red regions of the visible spectrum, with each layer having associated therewith a color-forming compound which, respectively, yields a yellow, magenta or cyan dye. The quality of the resulting color image is primarily based on the dye hues obtained from the respective color-forming compounds.

Dye image-forming coupler compounds are frequently employed to provide desired color images. A problem encountered with such couplers is that the spectral absorption characteristics of dyes obtained therefrom may not be in the particular narrow region where absorption is most desired. Frequently, the hue which is obtained may be as little as several nanometers removed from the optimum desired absorption value, and therefore be rejected for commercial use notwithstanding this slight difference. Conversely, a resulting dye may have an absorption maximum which is considerably shorter than a desired value.

Attempts to alter absorption characteristics of dyes obtained from dye image-forming coupler compounds are usually focused on alterations of the structures of coupler compounds. This approach, while enjoying some measure of success, is not only time consuming, but also involves the expense of highly focused research programs. Success with such programs is not predictable so that improvements in final hue values have been elusive, even after concentrated research efforts.

Some coupler solvents are known to cause shifts in absorption values of dyes. For example, U. S. Patent 3,676,137 describes use of a phosphate ester of a high boiling coupler solvent to shift absorption of a cyan dye to a shorter wavelength in order to reduce excessive red wavelength absorption. Alternatively, shifting absorption of a pyrazolone azomethine dye to a longer wavelength by use of a phenolic compound is known from Journal of the American Chemical Society, 73, 919 (1951).

Japanese Patent Publication No. 59(1984) - 204041 describes use of sulfamide compounds with cyan dye image-forming couplers to improve light fastness, to reduce unwanted green absorption and to reduce loss of density caused by bleach operations in dyes obtained from such couplers. This publication also suggests addition of other compounds that form dyes by oxidative coupling with primary amine color developing agents, such as magenta and yellow coupler compounds. However, there is no teaching or suggestion in this publication that a sulfonamide compound can be used to alter absorption characteristics of dyes derived from dye image-forming couplers or that particular compounds employed in this invention would be useful for this purpose.

European specification 0,264,083 (published 20 April 1988) describes the use of amines with cyan couplers and, as a subclass thereof sulphonamide compounds of the formula

R⁹-NHSO₂-R¹⁰

wherein R⁹ and R¹⁰ are each an alkyl or aryl group to obtain improved Dₘₐₓ, improved keeping of image dye, shifting λₘₐₓ and improved Dₘₐₓ without the use of benzyl alcohol in the color developer solution.

The object of the present invention is to provide a color photographic silver halide recording material having the capability of imparting slight as well as relatively large alterations in the absorption properties of a dye to obtain a desired spectral absorption which is different from the inherent absorption characteristics of the dye.

This object is achieved with a color photographic recording material which comprises a support having thereon a light-sensitive silver halide emulsion layer, a dye image-forming coupler capable of forming a dye by reaction with oxidized color developing agent and associated with the coupler, a sulfonamide compound which is capable of altering the spectral absorption of a dye formed from the coupler, said sulfonamide compound having the structural formula:

R¹SO₂NHR²

wherein:
R¹ and R² are substituted or unsubstituted alkyl having from 1 to 20 carbon atoms or phenyl which may be substituted with alkyl having from 1 to 4 carbon atoms or with sulfamoyl having the formula - SO₂NHR³ wherein R³ is alkyl of from 1 to 12 carbon atoms, or with halogen, wherein at least one of R¹ or R² is phenyl.
This invention also relates to a color photographic record comprising a dye formed by a coupling reaction between a dye image-forming coupler and oxidized silver halide developing agent, which recording material comprises, in association with the dye, a sulfonamide compound having the structural formula:

R¹SO₂NHR²

wherein;
R¹ and R² are as defined above.
Alkyl groups which are represented by R¹ and R² preferably have from about 1 to about 12 carbon atoms. The carbon chain can be straight or branched and can be substituted.

The type of substituents which can be present on the alkyl groups include hydroxy, halogen atoms, particularly chlorine and bromine or - SO₂R³ wherein R³ is as described above.

Chlorine is a preferred halogen substituent on a phenyl group inasmuch as it provides good stability properties and is least expensive to manufacture.

The described sulfonamide compounds are readily synthesized by reacting a sulfonyl chloride compound of the formula R¹SO₂Cl with ammonia or with a primary amine compound of the formula R²NH₂, according to procedures well known in the art. R¹ and R² have the meanings as described above.

There are no particular restrictions on the quantity of a sulfonamide compound which can be employed with a dye image-forming coupler either alone or in combination with known coupler solvents. Generally, it is desirable that the quantity of sulfonamide compound, with respect to each part by weight of coupler, be from about 0.05 to about 10 parts, preferably from about 0.2 to about 3 parts by weight of coupler compound. As the amount of sulfonamide compound increases, relative to the amount of coupler compound employed, there is usually a detectable increase in the extent of hue shift in the dye. However, the particular choice of coupler, of sulfonamide compound or the presence of one or more coupler solvents, all tend to influence the type and the extent of spectral absorption change in the resulting dye.

When the coupler compound is added to a silver halide emulsion, conventional procedures may be employed. For example, the coupler can first be dissolved in one or more known coupler solvents, such as di-n-butyl phthalate (DBP), and then be mixed with a sulfonamide compound as described herein. If desired, the coupler compound can be mixed with a sulfonamide compound, where these compounds are sufficiently compatible, so that known coupler solvents may not be needed. The resulting mixture or solution is then dispersed in aqueous gelatin, preferably containing a surfactant, and the dispersion is added to a silver halide emulsion which can then be coated by known techniques.

Specific sulfonamide compounds which are useful for shifting absorption values of dyes obtained by the reaction of dye image-forming coupler compounds with oxidized color developing agents include the following:

Couplers which form cyan dyes upon reaction with oxidized color developing agents are described in such representative patents and publications as U. S. Patent Nos. 2,474,293; 2,772,162, 2,801,171; 2,895,826; 3,002,836; 3,419,390; 3,476,563; 3,779,763; 3,996,253; 4,124,396; 4,248,962; 4,254,212; 4,296,200; 4,333,999; 4,443,536; 4,457,559; 4,500,635 and 4,526,864.

Preferred cyan coupler structures are phenols and naphthols which form cyan dyes on reaction with oxidized color developing agent. These preferred structures include the following moieties:
where R⁴ represents a ballast group, R⁵ represents one or more halogen atoms (e.g., chloro, fluoro), lower alkyl (e.g., methyl, ethyl, butyl) or lower alkoxy (e.g., methoxy, ethoxy, butoxy) groups and X is hydrogen or a coupling off group. An especially preferred R⁴ group on a C-3 type structure is
as described in U.S. Patent 4,333,999.
Couplers which form magenta dyes upon reaction with oxidized color developing agents are described in such representative patents and publications as: U.S. Patent Nos. 1,969,479; 2,311,082; 2,343,703; 2,369,489; 2,600,788; 2,908,573; 3,061,432; 3,062,653; 3,152,896; 3,519,429; 3,725,067; 4,120,723; 4,500,630;
4,540,654 and 4,581,326; and European Patent Publication Nos. 170,164 and 177,765; and copending U.S. Application Serial Numbers 23,517 of S. Normandin et al; 23,518 of R. Romanet et al; 23,519 of A. Bowne et al and 23,520 of A. Bowne et al, all filed March 9, 1987.

Preferred magenta couplers include pyrazolones compounds having the structural formulae:
pyrazolotriazole compounds having the structural formulae:
pyrazolobenzimidazole compounds having the structural formulae:
and indazole compounds having the structural formula:
wherein
X is as defined above;
R⁴ is a ballast group;
R⁶ is halogen (e.g., chloro, fluoro), alkyl or alkoxy having from 1 to 4 carbon atoms, phenyl or substituted phenyl (e.g., 2,4,6-trihalophenyl);
R⁷ is hydrogen or a monovalent organic radical, for example a saturated or unsaturated alkyl group having from 1 to about 20 carbon atoms (methyl, ethyl, propyl, butyl, decyl, dodecyl, heptadecyl, octadecyl); a cycloalkyl group (e.g. cyclohexyl); an aralkyl group (e.g. benzyl); an aryl group (e.g. phenyl, alkoxyphenyl in which the alkyl or alkoxy radical has from 1 to about 20 carbon atoms, nitrophenyl, aminophenyl, acylaminophenyl, alkylaminophenyl, naphthyl, diphenyl, diphenylether, diphenylthioether); a heterocyclic group (e.g. α-furyl, α-benzofuryl, α-pyridyl); an amino, hydroxy or carboxylic acid group, it being possible for the hydrogen atoms of these groups to be substituted, for instance by a mono- or dialkylamino group in which the alkyl groups have from 1 to about 20 carbon atoms; a cycloalkylamino group; an amino group in which one hydrogen atom is replaced by a pyrazolo-[1,5-a]-benzimidazolyl radical which is bonded in 3- position to said nitrogen atom so that couplers result in which two pyrazolo-[1,5-a]-benzimidazolyl radicals are connected by an amino group, and in which the remaining hydrogen atom may be replaced by a substituent such as an alkyl-, aryl-, aralkyl- or acyl- radical; an acylamino group in which the acyl radical is derived from an aliphatic, aromatic or heterocyclic carboxylic acid; a carboxylic acid group which is esterified by means of an aliphatic, cycloaliphatic or aromatic alcohol or by an aromatic compound having a phenolic hydroxy group; or a carboxyamido group in which the amido group may be substituted for example by a saturated or unsaturated alkyl, aralkyl, aryl or heterocyclic group;
R⁸ represents a hydrogen atom, a sulphonic acid or a carboxylic acid group; a halogen atom (e.g. chlorine or bromine); or an azo radical -N=NR¹³, wherein R¹³ can be an aromatic or heterocyclic radical (phenyl, naphthyl, diphenyl, diphenylether, benzthiazolyl, pyridyl, quinolyl or pyrazolyl) which may be substituted such as by an alkyl group having from 1 to about 20 carbon atoms, hydroxy, alkoxy, halogen, amino, substituted amino, nitro, sulphonic acid or carboxylic acid groups;
R⁹ represents a divalent radical such as
wherein R¹⁰ can be alkyl, aralkyl, especially phenyl, phenyl substituted preferably in the p-position by a tertiary amino group such as a dialkylamino group in which at least one of the alkyl groups is substituted by carboxy, sulpho, hydroxy, alkoxy, carboxylalkyl, cyano or the divalent radical
wherein R¹¹ and R¹² represent aliphatic, aromatic, araliphatic or heterocyclic radicals.

Specific magenta dye forming coupler compounds which are useful in the practice of this invention include:

Couplers which form yellow dyes upon reaction with oxidized color developing agent are described in such representative U. S. Patents as Nos. 2,298,443; 2,875,057; 2,407,210; 3,265,506; 3,384,657; 3,408,194; 3,415,652; 3,447,928; 3,542,840; 4,046,575; 3,894,875; 4,095,983; 4,182,630; 4,203,768; 4,221,860; 4,326,024; 4,401,752; 4,443,536; 4,529,691; 4,587,205; 4,587,207 and 4,617,256.

Preferred yellow dye image-forming couplers are acylacetamides, such as benzoylacetanilides and pivalylacetanilides. Structures of such preferred coupler moieties are:
where R¹³ is as defined above, R¹⁴ is hydrogen or one or more halogen, lower alkyl (e.g. methyl, ethyl) or a ballast (e.g. alkoxy of 16 to 20 carbon atoms) group and X is a coupling off group.

Photographic elements in which the photographic couplers of this invention are incorporated can be simple elements comprising a support and a single silver halide emulsion layer, or they can be multilayer, multicolor elements. The coupler compounds of this invention can be incorporated in the silver halide emulsion layer or in another layer, such as an adjacent layer, where they will come into reactive association with oxidized color developing agent which has developed silver halide in the emulsion layer. The silver halide emulsion layer can contain, or have associated therewith other photographic coupler compounds, such as color forming couplers, colored masking couplers, etc. These other photographic coupler compounds can form dyes of the same or different color and hue as the photographic coupler compounds of this invention. Additionally, the silver halide emulsion layer can contain addenda conventionally contained in such layers.

A typical multilayer, multicolor photographic element according to this invention comprises a support having thereon a red-sensitive silver halide emulsion layer have associated therewith a cyan dye image-forming coupler compound, a green-sensitive silver halide emulsion layer having associated therewith a magenta dye image-forming coupler compound and a blue-sensitive silver halide emulsion layer having associated therewith a yellow dye image-forming coupler compound, wherein at least one of the dye image-forming coupler compounds has associated therewith a sulfonamide compound as described herein. Each silver halide emulsion layer can be composed of one or more layers and the layers can be arranged in different locations with respect to one another. Typical arrangements are described in U.S. Patent Nos. 3,227,554; 3,620,747; 3,843,369; and 4,400,463 and in U.K. Patent No. 923,045.

The light sensitive silver halide emulsions can include coarse, regular or fine grain silver halide crystals or mixtures thereof and can be comprised of such silver halides as silver chloride, silver bromide, silver bromoiodide, silver chlorobromide, silver chloroiodide, silver chlorobromoiodide and mixtures thereof. The emulsions can be negative-working or direct-positive emulsions. They can form latent images predominantly on the surface of the silver halide grains or predominantly on the interior of the silver halide grains. They can be chemically and spectrally sensitized. The emulsions typically will be gelatin emulsions although other hydrophilic colloids can be used in accordance with usual practice.

The support can be of any suitable material used with photographic elements. Typically, a flexible support is employed, such as a polymeric film or paper support. Such supports include cellulose nitrate, cellulose acetate, polyvinylacetal, polyethylene terephthalate, polycarbonate and resinous materials as well as glass, paper or metal. Paper supports can be acetylated or coated with baryta and/or an α-olefin polymer, particularly a polymer of an α-olefin containing 2 to 10 carbon atoms such as polyethylene, polypropylene or ethylene-butene copolymers.

Further details regarding silver halide emulsions and elements, and addenda incorporated therein can be found in Research Disclosure, December 1971, Item 9232, Paragraphs I through XVIII. Research Disclosure is published by Industrial Opportunities Ltd., Homewell, Havant, Hampshire, P09 1EF, United Kingdom.

The terms "in association" or "associated with" are intended to mean that materials can be in either the same or different layers, so long as the materials are accessible to one another.

The following examples further illustrate the invention. Unless otherwise indicated all parts, percents and ratios are by weight.

### EXAMPLE I

Photographic elements employing coupler chemistry to show hue shifting with a 1-aryl-3-anilino-5-pyrazolone coupler and various sulfonamide compounds were prepared by coating on a paper support a silver chlorobromide emulsion layer (15 mole % chloride) comprising green sensitized 0.3 µm grains (0.42 gAg/m²). Each layer also contained gelatin (1.6 g/m²) and the magenta coupler M-1 (0.52 g/m²) as described above, dispersed in the coupler solvent di-n-butylphthalate (DBP) (0.52 g/m² when used alone) or in combination with DBP and a sulfonamide compound (SC), each at 0.26 g/m² as described below in Table I.

Each coating was exposed imagewise through a graduated-density test object to provide a maximum density image and was processed at 33°C employing the color developer solution described below, and then subjected to 1.5 minutes in the bleach-fix bath described below, washed and dried.

| Color Developer (pH 10.08) | |
|---|---|
| Triethanolamine | 11 mL |
| Benzyl alcohol | 14.2 mL |
| Lithium chloride | 2.1 g |
| Potassium bromide | 0.6 g |
| Hydroxylamine sulfate | 3.2 g |
| Potassium sulfite (45% solution) | 2.8 mL |
| 1-Hydroxyethylene-1,1-diphosphoric acid (60%) | 0.8 mL |
| 4-Amino-3-methyl-N-ethyl-N-β-methanesulfonamido)ethylaniline sulfate hydrate | 4.35 g |
| Potassium carbonate (anhydrous) | 28 g |
| Water to make | 1.0 liter |

| Bleach-Fix Bath (pH 6.8) | |
|---|---|
| Ammonium thiosulfate | 104 g |
| Sodium hydrogen sulfite | 13 g |
| Ferric ammonium ethylenediamine tetraacetic acid | 65.6 g |
| Ethylenediamine tetraacetic acid | 6.56 g |
| Ammonium hydroxide (28%) | 27.9 mL |
| Water to make | 1 liter |

Transmission density versus wavelength data were obtained to determine the λmax of the dye in an environment with the addition of different sulfonamide compounds. Results are recorded in Table I which reflects the coupler: DBP: sulfonamide compound (SC) ratio used in each test.

**Table I**

| Sulfonamide Compound | Weight Ratio Coupler:DBP:SC | λmax, nm |
|---|---|---|
| None(control) | 2 : 2 : 0 | 540 |
| 1 | 2 : 1 : 1 | 542 |
| 7 | 2 : 1 : 1 | 542 |
| 11 | 2 : 1 : 1 | 542 |
| 14 | 2 : 1 : 1 | 544 |
| 15 | 2 : 1 : 1 | 543 |

As is demonstrated by the data in Table I, hue shifts are highly subtle and vary only a few nanometers from the control when using sulfonamide compounds as described herein. These variations in wavelength shifts offer a high degree of manipulative control and provide an excellent, inexpensive means to obtain particularly desired hue values.

### EXAMPLE 2 - Tests using preformed dyes.

A solution of 6.25% photographic grade gelatin and 0.2% duPont Alkanol XC were added to each solution of preformed dye in 1ml ethyl acetate with coupler solvent di-n-butylpthalate (DBP) or sulfonamide compound (SC) or a mixture of DBP and SC. The dyes and the sulfonamide compounds are described below. The amounts used of each are shown in Table II.

This mixture was passed five times through a colloid mill and 0.2 ml (10% solution) Olin Corp. 10G surfactant and 0.05 ml (5.0% solution) formaldehyde were added. The milled mixture was then coated on a poly(ethyleneterephthalate) support, 100 µm wet thickness, and dried at 49°C. After 24 hours, the coating was washed for 5 minutes, dried, and spectrophotometric absorption maxima values were obtained.

Table II shows that sulfonamide compounds as described herein, are capable of shifting the absorption maxima of dyes derived from dye-forming couplers to usefully longer wavelengths. The extent of hue shifting depends upon the specific dye and sulfonamide compounds used and also varies with the dye: sulfonamide compound ratio. The Table reflects the Dye:DBP:sulfonamide compound (SC) ratio used in each test.

**Table II**

| Dye Compound* | Sulfonamide Compound(SC) | Weight Ratio Dye:DBP:SC | λ-max, nm |
|---|---|---|---|
| A | none(control) | 1 : 3 : 0 | 532 |
| A | 1 | 1 : 2 : 1 | 535 |
| A | 1 | 1 : 0 : 3 | 539 |
| A | 2 | 1 : 2 : 1 | 533 |
| B | none(control) | 1 : 3 : 0 | 533 |
| B | 1 | 1 : 0 : 3 | 543 |
| C | none(control) | 1 : 3 : 0 | 639 |
| C | 1 | 1 : 2 : 1 | 645 |
| C | 1 | 1 : 0 : 3 | 653 |
| C | 2 | 1 : 2 : 1 | 644 |

As is demonstrated by the data in Table II, hue shifts to longer wavelengths, varying from a few nanometers to as much as 14 nanometers, are possible with sulfonamide compounds as described herein. These variations in wavelength shifts offer a high degree of manipulative control and provide an excellent, inexpensive means to obtain particularly desired hue values with a variety of dye types.

## Claims (Claims for the following Contracting State(s): AT, BE, CH, ES, GR, LI, LU, SE)

1. A color photographic recording material comprising a support having thereon a light-sensitive silver halide emulsion layer, a dye image-forming coupler capable of forming a dye by reaction with oxidized color developing agent and, associated with the coupler, a sulfonamide compound which is capable of altering the spectral absorption of a dye formed from the coupler, said sulfonamide compound has the structural formula:
R¹SO₂NHR²
wherein;
R¹ and R² are a substituted or unsubstituted alkyl having from 1 to 20 carbon atoms or phenyl which may be substituted with alkyl having from 1 to 4 carbon atoms or with sulfamoyl having the formula - SO₂NHR³, where R³ is alkyl of from 1 to 12 carbon atoms, or with halogen, wherein at least one of R¹ or R² is phenyl.

2. A photographic recording material according to claim 1 wherein R¹ or R² is an alkyl group having from 1 to 12 carbon atoms.

3. A photographic recording material according to claim 1 wherein at least one of R¹ and R² comprises a halogen substituent.

4. A photographic recording material according to claim 3 wherein the halogen is chlorine.

5. A photographic recording material according to claim 1 wherein the sulfonamide compound is present in an amount of from about 0.05 to 5, preferably 0.3 to 3, parts by weight of coupler compound.

6. A photographic recording material according to claim 1 or 5 wherein the sulfonamide compound has the structural formula:

7. A photographic recording material according to claim 1 wherein the dye image-forming coupler is a magenta or cyan coupler.

8. A photographic recording material according to claim 7 wherein the dye is formed from a pyrazolone, or indazole magenta coupler compound.

9. A color photographic record comprising a dye formed by a coupling reaction between a dye image-forming coupler and oxidized silver halide developing agent, which recording material comprises, in association with the dye, a sulfonamide compound as specified in any of claims 1 to 8.

## Claims (Claims for the following Contracting State(s): DE, FR, GB, IT, NL)

1. A color photographic recording material comprising a support having thereon a light-sensitive silver halide emulsion layer, a dye image-forming coupler capable of forming a dye by reaction with oxidized color developing agent other than a cyan coupler and, associated with the coupler, a sulfonamide compound which is capable of altering the spectral absorption of a dye formed from the coupler, said sulfonamide compound has the structural formula:
R¹SO₂NHR²
wherein;
R¹ and R² are a substituted or unsubstituted alkyl having from 1 to 20 carbon atoms or phenyl which may be substituted with alkyl having from 1 to 4 carbon atoms or with sulfamoyl having the formula - SO₂NHR³, where R³ is alkyl of from 1 to 12 carbon atoms, or with halogen, wherein at least one of R¹ or R² is phenyl.

2. A photographic recording material according to claim 1 wherein R¹ or R² is an alkyl group having from 1 to 12 carbon atoms.

3. A photographic recording material according to claim 1 wherein at least one of R¹ and R² comprises a halogen substituent.

4. A photographic recording material according to claim 3 wherein the halogen is chlorine.

5. A photographic recording material according to claim 1 wherein the sulfonamide compound is present in an amount of from about 0.05 to 5, preferably 0.3 to 3, parts by weight of coupler compound.

6. A photographic recording material according to claim 1 or 5 wherein the sulfonamide compound has the structural formula:

7. A photographic recording material according to claim 1 wherein the dye image-forming coupler is a magenta coupler.

8. A photographic recording material according to claim 7 wherein the dye is formed from a pyrazolone, or indazole magenta coupler compound.

9. A color photographic record comprising a dye formed by a coupling reaction between a dye image-forming coupler and oxidized silver halide developing agent other than a cyan dye, which recording material comprises, in association with the dye, a sulfonamide compound as specified in any of claims 1 to 8.

## Patentansprüche (Patentansprüche für folgende(n) Vertragsstaat(en): AT, BE, CH, ES, GR, LI, LU, SE)

1. Farbphotographisches Aufzeichnungsmaterial mit einem Träger, auf dem sich befinden eine lichtempfindliche Silberhalogenidemulsionsschicht, ein ein Farbstoffbild bildender Kuppler, der einen Farbstoff durch Umsetzung mit oxidierter Farbentwicklerverbindung zu bilden vermag, und assoziiert mit dem Kuppler eine Sulfonamidoverbindung, die die spektrale Absorption des Farbstoffes, der aus dem Kuppler gebildet wurde, zu verändern vermag, wobei die Sulfonamidoverbindung der folgenden Strukturformel entspricht:
R¹SO₂NHR²
worin bedeuten:
R¹ und R² ein substituiertes oder unsubstituiertes Alkyl mit 1 bis 20 Kohlenstoffatomen oder Phenyl, das substituiert rein kann durch Alkyl mit 1 bis 4 Kohlenstoffatomen oder durch Sulfamoyl der Formel -SO₂NHR³, worin R³ Alkyl mit 1 bis 12 Kohlenstoffatomen darstellt oder durch Halogen, wobei mindestens R¹ oder R² für Phenyl steht.

2. Photographisches Aufzeichnugnsmaterial nach Anspruch 1, worin R¹ oder R² eine Alkylgruppe mit 1 bis 12 Kohlenstoffatomen darstellt.

3. Photographisches Aufzeichnungsmaterial nach Anspruch 1, in dem mindestens einer von R¹ und R² einen Halogensubstituenten umfaßt.

4. Photographisches Aufzeichnungsmaterial nach Anspruch 3, worin das Halogen Chlor ist.

5. Photographisches Aufzeichnungsmaterial nach Anspruch 1, in dem die Sulfonamidoverbindung in einer Menge von etwa 0,05 bis 5, vorzugsweise 0,3 bis 3 Gewichtsteilen, bezogen auf die Kupplerverbindung, vorliegt.

6. Photographisches Aufzeichnungsmaterial nach Anspruch 1 oder 5, in dem die Sulfonamidoverbindung der folgenden Strukturformel entspricht:

7. Photographisches Aufzeichnungsmaterial nach Anspruch 1, in dem der ein Farbstoffbild bildende Kuppler ein Purpurrot- oder Blaugrün-Kuppler ist.

8. Photographisches Aufzeichnungsmaterial nach Anspruch 7, in dem der Farbstoff aus einer Pyrazolon- oder Indazol-Purpurrot-Kupplerverbindung erzeugt worden ist.

9. Farbphotographische Aufzeichnung mit einem Farbstoff, der durch eine Kupplungsreaktion zwischen einem ein Farbstoffbild liefernden Kuppler und oxidierter Silberhalogenidentwicklerverbindung erzeugt worden ist, wobei das Aufzeichnungsmaterial in Assoziation mit dem Farbstoff eine Sulfonamidoverbindung nach einem der Ansprüche 1 bis 8 umfaßt.

## Patentansprüche (Patentansprüche für folgende(n) Vertragsstaat(en): DE, FR, GB, IT, NL)

1. Farbphotographisches Aufzeichnungsmaterial mit einem Träger, auf dem sich befinden eine lichtempfindliche Silberhalogenidemulsionsschicht, ein ein Farbstoffbild bildender Kuppler, der einen Farbstoff durch Umsetzung mit oxidierter Farbentwicklerverbindung zu bilden vermag und ein anderer Kuppler als ein blaugrüner Kuppler ist, und assoziiert mit dem Kuppler eine Sulfonamidoverbindung, die die spektrale Absorption des Farbstoffes, der aus dem Kuppler gebildet wurde, zu verändern vermag, wobei die Sulfonamidoverbindung der folgenden Strukturformel entspricht:
R¹SO₂NHR²
worin bedeuten:
R¹ und R² ein substituiertes oder unsubstituiertes Alkyl mit 1 bis 20 Kohlenstoffatomen oder Phenyl, das substituiert sein kann durch Alkyl mit 1 bis 4 Kohlenstoffatomen oder durch Sulfamoyl der Formel -SO₂NHR³, worin R³ Alkyl mit 1 bis 12 Kohlenstoffatomen darstellt oder durch Halogen, wobei mindestens R¹ oder R² für Phenyl steht.

2. Photographisches Aufzeichnugnsmaterial nach Anspruch 1, worin R¹ oder R² eine Alkylgruppe mit 1 bis 12 Kohlenstoffatomen darstellt.

3. Photographisches Aufzeichnungsmaterial nach Anspruch 1, in dem mindestens einer von R¹ und R² einen Halogensubstituenten umfaßt.

4. Photographisches Aufzeichnungsmaterial nach Anspruch 3, worin das Halogen Chlor ist.

5. Photographisches Aufzeichnungsmaterial nach Anspruch 1, in dem die Sulfonamidoverbindung in einer Menge von etwa 0,05 bis 5, vorzugsweise 0,3 bis 3 Gewichtsteilen, bezogen auf die Kupplerverbindung, vorliegt.

6. Photographisches Aufzeichnungsmaterial nach Anspruch 1 oder 5, in dem die Sulfonamidoverbindung der folgenden Strukturformel entspricht:

7. Photographisches Aufzeichnungsmaterial nach Anspruch 1, in dem der ein Farbstoffbild bildende Kuppler ein Purpurrot-Kuppler ist.

8. Photographisches Aufzeichnungsmaterial nach Anspruch 7, in dem der Farbstoff aus einer Pyrazolon- oder Indazol-Purpurrot-Kupplerverbindung erzeugt worden ist.

9. Farbphotographische Aufzeichnung mit einem Farbstoff, der durch eine Kupplungsreaktion zwischen einem ein Farbstoffbild liefernden Kuppler und oxidierter Silberhalogenidentwicklerverbindung erzeugt worden ist und ein anderer Farbstoff als ein blaugrüner Farbstoff ist, wobei das Aufzeichnungsmaterial in Assoziation mit dem Farbstoff eine Sulfonamidoverbindung nach einem der Ansprüche 1 bis 8 umfaßt.

## Revendications (Revendications pour l'(les) Etat(s) contractant(s) suivant(s): AT, BE, CH, ES, GR, LI, LU, SE)

1. Produit d'enregistrement photographique en couleurs comprenant un support recouvert d'une couche d'émulsion aux halogénures d'argent sensible à la lumière, un coupleur formateur d'image de colorant capable de former un colorant en réagissant avec un développateur chromogène oxydé et, associé à ce coupleur, un composé sulfonamide capable de modifier l'absorption spectrale du colorant formé à partir du coupleur, le composé sulfonamide ayant la formule :
R¹SO₂NHR²
où
R¹ et R² sont des radicaux alkyle substitués ou non ayant de 1 à 20 atomes de carbone ou un radical phényle qui peut être substitué par un alkyle de 1 à 4 atomes de carbone ou par un sulfamoyle de formule -SO₂NHR³, où R³ est alkyle de 1 à 12 atomes de carbone, ou par un halogène, où au moins l'un des groupes R¹ ou R² est phényle.

2. Produit d'enregistrement photographique selon la revendication 1 où au moins R¹ ou R² est un groupe alkyle de 1 à 12 atomes de carbone.

3. Produit d'enregistrement photographique selon la revendication 1 dans lequel au moins l'un des groupes R¹ et R² comprend un substituant halogène.

4. Produit d'enregistrement photographique selon la revendication 3 où l'halogène est le chlore.

5. Produit d'enregistrement photographique selon la revendication 1 où le composé sulfonamide et présent à raison de 0,05 à 5 et de préférence 0,3 à 3 parties en poids de composé coupleur.

6. Produit d'enregistrement photographique selon la revendication 1 ou 5 où le composé sulfonamide a la formule :

7. Produit d'enregistrement photographique selon la revendication 1 où le coupleur formateur d'image de colorant est un coupleur magenta ou cyan.

8. Produit d'enregistrement photographique selon la revendication 7 où le colorant est formé à partir d'un composé coupleur pyrazolone ou indazole magenta.

9. Enregistrement photographique en couleurs comprenant un colorant formé par une réaction de couplage entre un coupleur formateur d'image de colorant et un développateur des halogénures d'argent oxydé, enregistrement comprenant en association avec le colorant, un composé sulfonamide tel que spécifié dans l'une quelconque des revendications 1 à 8.

## Revendications (Revendications pour l'(les) Etat(s) contractant(s) suivant(s): DE, FR, GB, IT, NL)

1. Produit d'enregistrement photographique en couleurs comprenant un support recouvert d'une couche d'émulsion aux halogénures d'argent sensible à la lumière, un coupleur formateur d'image de colorant capable de former un colorant en réagissant avec un développateur chromogène oxydé autre qu'un coupleur cyan et associé à ce coupleur, un composé sulfonamide capable de modifier l'absorption spectrale du colorant formé à partir du coupleur, le composé sulfonamide ayant la formule :
R¹SO₂NHR²
où
R¹ et R² sont des radicaux alkyle substitués ou non ayant de 1 à 20 atomes de carbone ou un radical phényle qui peut être substitué par un alkyle de 1 à 4 atomes de carbone ou par un sulfamoyle de formule -SO₂NHR³, où R³ est alkyle de 1 à 12 atomes de carbone, ou par un halogène, où au moins l'un des groupes R¹ ou R² est phényle.

2. Produit d'enregistrement photographique selon la revendication 1 où au moins R¹ ou R² est un groupe alkyle de 1 à 12 atomes de carbone.

3. Produit d'enregistrement photographique selon la revendication 1 dans lequel au moins l'un des groupes R¹ et R² comprend un substituant halogène.

4. Produit d'enregistrement photographique selon la revendication 3 où l'halogène est le chlore.

5. Produit d'enregistrement photographique selon la revendication 1 où le composé sulfonamide et présent à raison de 0,05 à 5 et de préférence 0,3 à 3 parties en poids de composé coupleur.

6. Produit d'enregistrement photographique selon la revendication 1 ou 5 où le composé sulfonamide a la formule :

7. Produit d'enregistrement photographique selon la revendication 1 où le coupleur formateur d'image de colorant est un coupleur magenta.

8. Produit d'enregistrement photographique selon la revendication 7 où le colorant est formé à partir d'un composé coupleur pyrazolone ou indazole magenta.

9. Enregistrement photographique en couleurs comprenant un colorant formé par une réaction de couplage entre un coupleur formateur d'image de colorant et un développateur des halogénures d'argent oxydé autre qu'un colorant cyan, enregistrement comprenant en association avec le colorant, un composé sulfonamide tel que spécifié, dans l'une quelconque des revendications 1 à 8.
